

O. A. HEPPES.

WATERPROOF AND AIRPROOF CARDBOARD AND PROCESS OF MAKING THE SAME.  
APPLICATION FILED DEC. 6, 1918.

1,320,549.

Patented Nov. 4, 1919.



WITNESSES:  
Robert F. Weir  
Arthur W. Carlson

Inventor  
Otto A. Heppes  
James Rain & Bean  
Atty5:

# UNITED STATES PATENT OFFICE.

OTTO A. HEPPES, OF LA GRANGE, ILLINOIS.

## WATERPROOF AND AIRPROOF CARDBOARD AND PROCESS OF MAKING THE SAME.

1,320,549.

Specification of Letters Patent. Patented Nov. 4, 1919.

Application filed December 6, 1918. Serial No. 265,506.

*To all whom it may concern:*

Be it known that I, Otto A. HEPPES, a citizen of the United States, residing at La Grange, in the county of Cook and State 5 of Illinois, have invented certain new and useful Improvements in Waterproof and Airproof Cardboard and Processes of Making the Same, of which the following is a specification.

10 My invention relates to a new and useful process of making water-proof and air-proof cardboard and cartons.

One of the objects of my invention is to provide a cheap and continuous process of 15 making water-proof and weather-proof cardboard, which is especially adaptable for stock in the manufacture of cartons, or the like, which are used for containing foods, or other perishable staples and products 20 that must be protected from contamination by air and dampness.

Another object of my invention is to provide a new process of making cartons and the like.

25 In the manufacture of cartons heretofore, a board, constituting the base, is cut or punched into the desired shape, to fashion into carton forms and after the carton has been made, it is then necessary to provide 30 an inner container, such as may be made of relatively thin and impervious paper, after which the outer surface of the carton is covered with another laminae of 35 paper, of a different character, and which provides a surface well adapted to receive the paper, whereupon the manufacturer has printed suitable indicia to identify the products and the manufacturer thereof. This last printed paper coating is pasted 40 over the cardboard face to provide a finish after the cardboard pattern has been cut from the sheet.

In preparing card board sheets of this 45 character, it has heretofore been customary to provide the base or stock by securing two relatively thin sheets of straw board, or like sheet stock, together, by a water and air proof adhesive, such, for example, as a thin coating of asphaltic plastic. This product 50 presents two rough, relatively unclean surfaces that are to be covered, in the manner heretofore described, when the stock is to be made up into cartons.

The inside surface of such cartons is not, 55 strictly, sanitary, hence the necessity for the inner container lining, and the outside

surface is not well adapted to receive the printers' ink and therefore a separate ink-receiving sheet must be printed and subsequently pasted on the outer surface of the 60 carton. These operations are necessarily expensive because they require hand manipulation and personal supervision.

In carrying my invention into effect I provide a roll of pervious, relatively heavy 65 board, such for example as strawboard, or the like, as indicated by 10 in the accompanying schematic drawing forming a part hereof. The board 10 is then passed through feed rollers 11 and 12 into a tank 70 13 in which is contained a heated solution of penetrable, relatively thin, asphalt 14, heated as by a furnace 15, to the proper temperature. A roller 16 causes continuous submergence of the sheet 10, after which 75 it is passed through the feed rollers 17 and 18 to the rollers 19 and 20. It is then passed into a tank 21 under a roller 22, which tank contains a solution of harder, less penetrable asphaltic material, which becomes thor- 80oughly water-proof when cool, and forms a continuous, unbroken, impervious coating on each side of the board 10. The asphalt 23 is heated by a fire 24 to the proper degree and as the sheet passes out of the tank 85 21 the excessive amount is scraped off by the doctors or scrapers 24 and 25, so as to provide a substantially uniformly thick hard coat on either side of the board. It is then passed between the rollers 26 and 90 27 and may be carried back over a roller 28 to increase the length to give it time to cool or become tacky. A blower 29, or other means, may be used for the purpose of cooling the sheet 10 as it passes back 95 over the roller 28 so that by the time it reaches the roller 30 it is in a tacky or sticky condition. It is then placed between spaced-apart rollers 31 and 32 to the feed rollers 33 and 34. As it passes through the 100 feed rollers a sheet of relatively thin paper, coming from the rollers 35 and 36, respectively, is pressed into contact, on either side of the continuous sheet or strip 10, and the asphaltic material, being in a tacky 105 condition and naturally of a cementitious character, the rollers 33 and 34 cause perfect adhesion between the thin paper strips 39 and 40 with the board 10. The strip 39 may be made of a relatively thin paper, 110 such as parchment, paraffin coated, or the like, and the strip 40 may be of a character

to receive printers' ink without permitting the asphalt to strike through. Therefore when the strip arrives, as at 41, it is coated on one side by a weather and air resisting paper and on the other side with a paper well adapted to receive printers' ink and which is of such character as to prevent the black asphalt from showing through.

After the product comes from the rollers, 10 33 and 34, it may be cut into the proper length and then punched out by suitable punches into patterns to form cartons, after which the pattern thus punched out may be printed before the pattern is formed into 15 carton shape. The other side of the carton blank is covered with a paper of parchment character, similar to that of which the inner containers of cartons heretofore described, are usually made. The character of paper 20 best adapted for this purpose may be used and which is of such nature as to prevent striking through of the asphaltic coating and yet be of a nature that will be sufficiently adhesive to adhere thereto.

25 In the products made, in the manner described, about 75 to 85 per cent. of the stock consists of the straw board, the penetrable solution of asphaltic character and the relatively hard layer of asphalt, on either side, 30 all of which are relatively cheap materials, the high grade or more expensive material consisting of the substantially impervious layer of paper on one side for the interior of the carton and the ink-receiving paper 35 on the opposite side constitute a very small proportion, in weight, of the whole structure and therefore it will be observed that my product is substantial, cheap and well adapted for the purpose intended.

40 In the making of the product, the sheets

of paper that overlie the asphaltic stock are half an inch, or more, wider at each edge than the stock itself, thus preventing excessive asphaltic material from oozing out between the sheets and reaching the outer 45 surface on either side.

After the stock material has passed through the mill and become cooled, it is then ready for use.

Having described my invention, what I 50 claim is:—

1. The art of making carton board which consists in passing a strip of relatively thick pervious board through a hot solution of penetrable asphaltic material; then depositing, on each side thereof, a uniform coating of relatively hard substantially impenetrable and impervious asphaltic material and while in a sticky, or tacky condition covering one side of said board with a relatively thin 60 parchment-like paper and simultaneously covering the other side with a relatively thin sheet of paper adapted to receive printers' ink; then applying pressure to the composite board to stick the members together and then cooling the finished product. 65

2. An article of manufacture, carton board stock, comprising a fibrous, pervious board base having incorporated therewith weather-proof, adhesive, penetrable asphaltic material; a thin parchment-like paper covering one side of the base and paper adapted to receive printers' ink and to prevent the asphalt from striking through covering the other side of said base, said papers being 70 75 bound to the base by the adhesive qualities of the asphalt.

In testimony whereof I hereunto subscribe my name.

OTTO A. HEPPE.